

# UNITED STATES PATENT OFFICE.

THOMAS C. MEADOWS, OF NEW YORK, N. Y.

## PROCESS OF PRODUCING HIGH-PHOSPHORUS PIG-IRON.

1,322,038.

Specification of Letters Patent. Patented Nov. 18, 1919.

No Drawing.

Application filed May 4, 1918. Serial No. 232,476.

*To all whom it may concern:*

Be it known that I, THOMAS C. MEADOWS, a citizen of the United States, residing at New York, in the county of New York and 5 State of New York, have invented new and useful Improvements in Processes of Producing High-Phosphorus Pig-Iron, of which the following is a specification.

This invention relates to a new and useful process of treating greensand or like materials containing iron and an alkali metal, particularly potassium.

The object of this invention is to provide a method which will be simple in its nature, 15 comparatively easy to carry out and less costly to operate than those heretofore proposed. With these and other objects in view the invention consists in the novel steps and combination of steps constituting the process 20 all as will be more fully hereinafter disclosed and particularly pointed out in the claims.

In carrying out this invention glauconite, commonly called greensand, phosphate rock, 25 and coke or other suitable fuel, are fed to a blast furnace.

In addition to high phosphorus pig iron, other valuable materials are recovered in the operation. These comprise potassium-nitrogen-carbon compounds.

Although I preferably employ a blast furnace I do not wish to be limited to this as other types, such as electric furnaces, etc., may be employed with more or less success 35 provided they are constructed and operated in such a manner that the reactions are substantially those normally occurring in a blast furnace.

In preparing the materials for charging, 40 briquetting or sintering may be resorted to especially in the case of greensand which has a tendency to dust and choke up a furnace.

As the material sought in my process is 45 essentially a high phosphorus pig iron the proportions of the various constituents of the charge are determined with this end in view. This necessitates either limiting the phosphate rock to a point where all of its 50 liberated phosphorus may be taken into combination by the iron of the greensand, or the total iron of the charge may be increased by the addition of iron ore, such as magnetite, etc., and especially varieties contaminated with apatite. Also if the charge is

deficient in acid or basic constituents respectively,  $\text{SiO}_2$  or  $\text{CaO}$  may be added.

Another method of increasing the iron content is by using phosphate rock high in iron. Such phosphate rock exists in abundance but is not now marketable because it cannot be economically employed in the acid process for fertilizer manufacture.

Although I have specified greensand I do not wish to be limited to this particular material as any potassium iron carrying material will answer the purpose, or any suitable mixture of materials containing these.

It has long been recognized that potassium-nitrogen-carbon compounds are formed 70 in the reaction zones of blast furnaces and play an important though little understood part in the general reactions. It has been stated that  $\text{KCN}$  is the agent that reduces  $\text{FeO}$  to  $\text{Fe}$  and that it is formed by the contact of potassium vapor and nitrogen in presence of incandescent carbon.

The amount of potassium normally occurring in blast furnace charges is very small occurring only as impurities in the charge. 80 In this invention the amount of potassium-nitrogen-carbon compounds is so considerable that a large part of same may be recovered by removing them from the reaction zone of the blast furnace before they are decomposed, without interfering with the production of the high phosphorus pig iron.

It is obvious that those skilled in the art may vary the details of the process as well as the proportions set forth, without departing from the spirit of the invention, and therefore I do not wish to be limited to the above disclosures except as may be required by the claims.

I claim:

1. A process of producing high phosphorus pig iron and nitrogen-potassium-carbon-compounds which comprises smelting greensand; phosphate rock; and fuel in a blast furnace; substantially as described. 100

2. A process of producing high phosphorus pig iron and nitrogen-potassium-carbon-compounds which comprises smelting greensand; phosphate rock; and coke in a blast furnace; periodically tapping off the molten high phosphorus iron; and continuously drawing off the vapor in the region immediately above the reaction zone of the furnace; substantially as described. 105

3. A process of producing high phos- 110

phorus pig iron and nitrogen-potassium-carbon-compounds which comprises smelting greensand; phosphate rock; and fuel in a blast furnace; tapping off the molten high phosphorus iron; and drawing off the vapors and suspended solids from the region immediately above the reaction zone; substantially as described.

4. A process of producing high phosphorus pig iron and nitrogen-potassium-carbon-compounds which comprises smelting greensand; phosphate rock; and fuel; tapping off the molten high phosphorus iron and drawing off the potassium-nitrogen-carbon compounds from the region immediately above the reaction zone; substantially as described.

5. A process of producing high phosphorus pig iron and nitrogen-potassium-carbon-compounds which comprises smelting greensand accompanied by additional iron ore; phosphate rock; and fuel; tapping off the molten high phosphorus iron; and drawing off the nitrogen-potassium-carbon compounds from the region imme-

diate above the reaction zone; substantially as described.

6. A process of producing high phosphorus pig iron and nitrogen-potassium-carbon-compounds which comprises smelting greensand enriched with other iron ore; phosphate rock; and fuel; substantially as described.

7. A process of producing high phosphorus pig iron and nitrogen-potassium-carbon-compounds which comprises smelting greensand; phosphate rock accompanied by a flux, and fuel, substantially as described.

8. A process of producing high phosphorus pig iron and nitrogen-potassium-carbon-compounds which comprises smelting greensand ore; phosphate rock associated with additional fluxing material; and fuel; tapping off the molten high phosphorus iron; and drawing off the nitrogen-potassium-carbon compounds from the region immediately above the reaction zone; substantially as described.

THOMAS C. MEADOWS.